

# UNITED STATES PATENT OFFICE.

PAUL RADMANN, OF GODEGÅRD, SWEDEN.

## METHOD OF PRODUCING SOLUBLE ALKALINE COMPOUNDS.

1,209,201.

Specification of Letters Patent. Patented Dec. 19, 1916.

No Drawing.

Application filed May 23, 1914. Serial No. 840,434.

To all whom it may concern:

Be it known that I, PAUL RADMANN, a subject of the King of Sweden, residing at Godegård, Sweden, have invented new and useful Improvements in Methods of Producing Soluble Alkaline Compounds, of which the following is a specification.

The present invention refers to a method of producing soluble alkali metal compounds (especially potassium compounds) from alkali-bearing rocks (especially feldspar) or devitrifying products.

The method consists in heating a suitable or proper mixture of the rock or devitrifying product and gypsum to a temperature falling below the temperature at which the mixture fuses. After this heating process the resulting mass contains the soluble alkali metal compounds in a condition allowing of their being easily separated or recovered, and the recovery of these alkali metal compounds is easily done *e. g.* by washing the mass with water.

The inventor is aware that it has previously been proposed to produce soluble alkali metal compounds by means of a mixture of feldspar and gypsum, but this was done by fusing the mixture. In so doing only a portion of the alkali metal compounds escapes in the form of gas and is recovered, whereas a greater or smaller portion, according to the temperature, remains in the fused mass. If the remaining alkali metal compounds are to be recovered by means of washing, the mass has first to be disintegrated by means of a special and separate process, but on account of the vitreous nature of the mass the gain is very small. With the known method and with the process here in question masses of quite a different nature are being obtained, and with the known process it is very probable that even by making use of three different operations, *viz.* the recovery of the alkali metal compounds escaping as vapor, the disintegration of the remainder of the mass and the washing of the same, no such good result will be obtained as by the single operation with the invention here referred to, *viz.* washing for instance. Furthermore the high temperatures required in connection with the known process for obtaining the best possible result offer great difficulties in obtaining a construction of furnace in which the material used for the construction is able to resist the influence of the fused mass and the

gases. With the process forming the object of this invention the mixture is not fused, and therefore does not affect or corrode the lining of the furnace. With this invention a practical process has therefore been obtained giving a good result. According to the present invention a suitable and proper proportion of limestone may also be added to the mixture. Tests carried out have proved that the best result is obtained if the mixture is finely pulverized to about the "fineness of cement". The mixture is then similar to flour or powder. The proper temperature in the process of this invention is between something like 1000 to 1250° C. As suitable proportions in the mixture may be mentioned 0.25 to 1 part by weight of gypsum, with or without the addition of up to 3 parts by weight of limestone, to 1 part by weight of feldspar. For such a mixture a heat of up to 1100 or 1250° C. is required.

In making practical use of the invention the time during which the heating process is going on may vary within wide limits, from one hour to several days, all dependent upon the nature of the devices used.

The following table shows the result of some tests made on the basis of the invention herein:

| Mixture—Parts in weight. |               |         | Temperature to which heated. | Alkali soluble in water in per cent. of the alkali in the feldspar. |
|--------------------------|---------------|---------|------------------------------|---------------------------------------------------------------------|
| Feldspar.                | Gypsum.       | Marble. |                              |                                                                     |
| 1                        | $\frac{1}{2}$ | —       | 1100                         | 30.4                                                                |
| 1                        | $\frac{1}{2}$ | —       | 1150                         | 33.9                                                                |
| 1                        | 1             | —       | 1100                         | 51.7                                                                |
| 1                        | 1             | —       | 1150                         | 58.7                                                                |
| 1                        | 1             | —       | 1200                         | 49.8                                                                |
| 1                        | $\frac{1}{2}$ | —       | 1150                         | 65.1                                                                |
| 1                        | $\frac{1}{2}$ | —       | 1200                         | 62.0                                                                |
| 1                        | $\frac{1}{2}$ | —       | 1150                         | 99.0                                                                |
| 1                        | $\frac{1}{2}$ | 3       | 1150                         | 100.0                                                               |

When mixing it ought to be seen to that the materials used are mixed as closely and carefully as possible. Afterward, when the alkali metal compounds have been washed out, the remainder of the mixture treated may be turned into cement, with or without the addition of limestone.

What I claim is:

1. A process of producing soluble alkali metal compounds from alkali-metal bearing rock consisting in heating a mixture of the said rock, gypsum, and limestone, in the proportion of one part by weight of rock, one half part by weight of gypsum, and

three parts by weight of limestone, to a temperature falling slightly below the fusing point of the mixture.

2. A process of producing soluble alkali metal compounds from alkali metal bearing rock consisting in heating a mixture of the said rock, gypsum, and limestone, in the proportions of one part by weight of rock, 0.25 to 1 part by weight of gypsum, and up to 3 parts by weight of limestone, to a temperature of 1100 to 1250 centigrade.

3. A process of producing soluble alkali-metal compounds from alkali-metal bearing

rock consisting in heating a mixture of the said rock, gypsum, and limestone, in the proportion of one part by weight of rock, one half part by weight of gypsum, and three parts by weight of limestone, to a temperature of 1150° centigrade.

In testimony whereof I have signed my name to this specification in the presence of two subscribing witnesses.

PAUL RADMANN.

Witnesses:

J. F. A. RUTRÄCK,  
M. LINDQUIST.